

Feb. 6, 1940.

B. R. F. KJELLGREN ET AL

2,188,904

METHOD OF PRODUCING METALLIC BERYLLIUM

Filed March 16, 1936



INVENTORS

BY  
Bengt R. F. Kjellgren  
Charles B. Sawyer  
Ray S. Zehr

ATTORNEY.

## UNITED STATES PATENT OFFICE

2,188,904

METHOD OF PRODUCING METALLIC  
BERYLLIUM

Bengt R. F. Kjellgren and Charles B. Sawyer,  
Cleveland Heights, Ohio, assignors to The Brush  
Beryllium Company, Cleveland, Ohio, a corpo-  
ration of Ohio

Application March 16, 1936, Serial No. 69,096

3 Claims. (Cl. 204—19)

This invention relates to an improved method of producing metallic beryllium from beryllium chloride by electrolysis of the said chloride in a molten bath.

5 Since beryllium chloride is a non-conductor of electricity it cannot be electrolyzed alone. To overcome this difficulty it was early proposed by W. Borchers (Zeitschrift für Electrochemie, vol. 2, 39, 1895) to electrolyze a melted mixture of beryllium chloride with alkaline chlorides or alkaline earth chlorides. Borchers carried out the electrolysis in a wrought iron crucible which at the same time served as the cathode with a carbon rod for the anode. The molten mixture 10 was heated with gas to a temperature just reaching the melting point of beryllium (1278° C.). As beryllium chloride boils at about 500° C. it is clear that the melt used by Borchers must have contained a substantially lessened amount of beryllium chloride. Since Borchers' work others 15 have electrolyzed melted mixtures of beryllium chloride and sodium chloride at temperatures of about 800° C. At this temperature also the losses of beryllium chloride due to volatilization are 20 considerable and in practice it would be necessary to recover the volatilized beryllium chloride in the interest of economy.

An object of the present invention is to provide a method of electrolysis of beryllium chloride in which losses due to volatilization are 25 eliminated or minimized at the temperature at which the electrolysis is carried out.

A further object of the invention is to minimize the amount of electrical energy consumed in the production of metallic beryllium by electrolysis through the use of heat from gas or other low-cost fuels for maintaining the electrolyte in a molten condition.

Another object of the invention is to overcome difficulties with the materials used in the construction of the electrolyzer, such as characterize methods of electrolysis at high temperatures.

Another object of the invention is the reduction of chemical attack on anodes, cathodes, and other parts of the electrolytic cell.

We have found it possible to produce mixtures of beryllium chloride with alkali chlorides or alkaline earth chlorides having freezing points not only below the boiling point of beryllium chloride (500° C.) but even far below the melting point of beryllium chloride (400° C.), and which mixtures in the molten state have adequate conductivity and other characteristics favorable for electrolysis. For example, to the eutectic mixture of potassium chloride, lithium

chloride and sodium chloride, which has a freezing point of 362° C., beryllium chloride may be added in varying proportions to produce a corresponding series of such low freezing point mixtures.

The freezing point of these mixtures are shown by the graph in the accompanying drawing. In this drawing ordinates represent centigrade melting temperatures and abscissas represent percentage proportions by weight of the beryllium chloride to the remainder of the electrolyte mixture. From the graph it will be noted that a mixture containing 50%  $BeCl_2$  and 50%  $KCl$ ,  $LiCl$ ,  $NaCl$  eutectic melts as low as 238° C. This mixture contains 20.2%  $LiCl$ , 26.6%  $KCl$ , 3.2%  $NaCl$  and 50%  $BeCl_2$ . The viscosity of this mixture at 260°—270° C. is sufficiently low to permit an efficient electrolysis.

It will be observed further from the graph of the drawing that combinations of the eutectic mixture with  $BeCl_2$  up to 50%  $BeCl_2$  have melting points ranging from about 238° C. to the relatively low temperature of 385° C. and are suitable for electrolysis at temperatures substantially below the boiling point of  $BeCl_2$ .

It is to be observed further, in connection with the graph of the drawing, that the melting point (362°) of the eutectic mixture of  $KCl$ ,  $LiCl$  and  $NaCl$  is not only far below the boiling point of beryllium chloride but also substantially below its melting point of about 400° C. Consequently the eutectic mixture can be prepared in the molten state and the beryllium chloride added thereto with practically no volatilization and loss of the beryllium chloride.

Another advantage of our low melting point eutectic mixture combined with beryllium chloride is that close regulation of the amount of beryllium chloride in the bath is not necessary since the electrolytic bath cannot be solidified even by electrolyzing out all of the beryllium chloride if the bath is maintained above about 385° C.

In carrying out our method of electrolysis it is not necessary to use the eutectic mixture of  $KCl$ ,  $LiCl$  and  $NaCl$ . The freezing points of various mixtures of these three salts and of three component mixtures of various other alkali salts and alkaline earth salts have heretofore been determined. In the International Critical Tables, Vol. IV, there are given three-component freezing point diagrams of the  $KCl$ ,  $LiCl$  and  $NaCl$  mixture and of various other alkaline chloride and alkaline earth chloride mixtures. Thus, from the proper diagram, proportions of melts of  $KCl$ ,  $LiCl$  and  $NaCl$  may be taken and anhydrous

BeCl<sub>2</sub> added to make mixtures with melting points below the boiling point of beryllium chloride. As BeCl<sub>2</sub> even at its melting point has a considerable vapor pressure it is desirable to 5 carry out the electrolysis below 400° C. but temperatures in the range of 450° C.-500° C. have been used without serious loss of BeCl<sub>2</sub> by volatilization.

Anhydrous beryllium chloride may also be 10 added to eutectic mixtures of other chlorides or to mixtures of such other chlorides having compositions sufficiently close to the eutectic mixture to have sufficiently low melting points for the purpose of carrying out our method. For example, we may use eutectic mixtures, or mixtures 15 approaching the eutectic compositions, as follows:

| 20                    | Composition of eutectic | Freezing point<br>°C. |
|-----------------------|-------------------------|-----------------------|
| 52% CaCl <sub>2</sub> |                         | 508                   |
| 48% NaCl              |                         |                       |
| 52% CaO <sub>2</sub>  |                         |                       |
| 6% KCl                |                         | 504                   |
| 25 42% NaCl           |                         |                       |
| 34% SrCl <sub>2</sub> |                         |                       |
| 36% NaCl              |                         | 504                   |
| 30% KCl               |                         |                       |
| 24% BaCl <sub>2</sub> |                         |                       |
| 41% KCl               |                         | 522                   |
| 35% NaCl              |                         |                       |

30 The foregoing eutectic mixtures serve only as examples of mixtures of alkali chlorides or alkaline earth chlorides that may be used with anhydrous beryllium chloride to produce melts 35 having melting points suitable for electrolyzing beryllium chloride below its boiling point. In this connection it is observed that, in order to secure the lowest melting points for the complete mixtures including the beryllium chloride, it may 40 be necessary to depart from the eutectic proportions of the other chlorides.

For the electrolyzer for carrying out our process a container made of ceramic material, porcelain, pyrex glass, or quartz may conveniently 45 be used. The low temperature at which the electrolysis is carried out makes possible the use of a much wider variety of such materials than would be possible at the higher temperature used in prior processes. The container may be 50 heated externally with a gas flame. The cathode may consist of a metal sheet of aluminum, copper, nickel or other suitable material. Graphite may be used for the anode as we have found that graphite is not noticeably attacked by 55 the chlorine released during electrolysis at the low electrolyte temperatures which we are able to employ.

By way of illustration and for the purpose of

more clearly explaining the invention we give the following description of one suitable procedure followed in carrying out our process:

796 grams KCl, 610 grams LiCl, 93 grams NaCl and 1500 grams BeCl<sub>2</sub> were melted in a quartz 5 container heated externally to about 300° C. One aluminum sheet cathode and two graphite plate anodes were used, the cathode being placed between the anodes so that beryllium was deposited on both sides of the cathode. The electrolysis lasted 24 hours, 20 minutes and the temperature varied between 290° C. and 326° C. The voltage required for the decomposition of the beryllium chloride was 2.2 volts and the current was about 1.78 amperes. 6.7 grams of metallic 10 beryllium crystals were produced with a current efficiency of 94.8%.

After the electrolysis is stopped the aluminum cathode may be lifted out of the bath and immersed in a cleansing solution which may consist of water with final drying in alcohol. 20

The above procedure may be varied widely in carrying out the invention, as will be apparent from the appended claims defining the scope of the invention. 25

What we claim is:

1. The process of producing metallic beryllium which comprises electrolyzing beryllium chloride from a molten bath consisting of beryllium chloride and a eutectic mixture of potassium chloride, lithium chloride and sodium chloride, the beryllium chloride constituting from 40% to 52% by weight of the bath. 30

2. The process of producing metallic beryllium which comprises forming a mixture made 35 up of approximately 50% by weight of beryllium chloride, 20.2% lithium chloride, 26.6% potassium chloride and 3.2% sodium chloride, and electrolyzing the beryllium chloride from a molten bath of the said mixture while the bath 40 is maintained at a temperature between 260° C. and 300° C.

3. The process of producing metallic beryllium which comprises adding anhydrous beryllium chloride to a mixture of lithium chloride, 45 potassium chloride and sodium chloride combined in substantially eutectic proportions and having a melting point below the melting point of anhydrous beryllium chloride, the beryllium chloride making up from about 30% to about 50 90% of all the materials, and electrolyzing the beryllium chloride from a bath of the combined materials while the bath is maintained in a molten state at temperatures below the boiling point of anhydrous beryllium chloride. 55

BENGT R. F. KJELLGREN.  
CHARLES B. SAWYER.